

# UNITED STATES PATENT OFFICE.

CLIFFORD A. WOODBURY, OF CHESTER, PENNSYLVANIA, ASSIGNOR TO E. I. DU PONT DE NEMOURS POWDER COMPANY, OF WILMINGTON, DELAWARE, A CORPORATION OF NEW JERSEY.

## EXPLOSIVE.

1,124,679.

Specification of Letters Patent.

Patented Jan. 12, 1915.

No Drawing. Application filed May 18, 1912, Serial No. 698,346. Renewed June 9, 1914. Serial No. 844,016.

To all whom it may concern:

Be it known that I, CLIFFORD A. WOODBURY, of Chester, in the county of Delaware, and in the State of Pennsylvania, have invented a certain new and useful Improvement 5 in Explosives, and do hereby declare that the following is a full, clear, and exact description thereof.

The object of my invention has been to 10 provide an explosive having approximately a specified velocity of detonation, and particularly a relatively low velocity of detonation, and to such ends my invention consists in the explosive hereinafter specified.

15 As an embodiment of my invention by which to illustrate its principle, I have chosen an explosive which is adapted for use in the mining of coal. Such explosive may have the following formula: nitrate of 20 ammonia 80%, nitro-glycerin 10%, absorbent (such as wood pulp) 10%.

An explosive of the above stated formula, using ammonium nitrate in the form ordinarily produced, has a relatively high velocity of detonation so that when used in the mining of coal it shatters the coal and breaks it up too small for sale as lump coal. The ammonium nitrate ordinarily used in explosives of this kind is so fine that from 25 50 to 90% will pass a 60-mesh sieve, and 25% or more would ordinarily pass a 100-mesh sieve. An explosive of the above composition made with this ordinary type of ammonia has a velocity of detonation of 30 35 from 3000 to 3600. I desire to produce an explosive having said formula but which has a low velocity of detonation so as to successfully produce lump coal. I have found that by making the said explosive of 40 ammonium nitrate having relatively coarse grains, I am able to reduce the velocity of detonation to the desired point. For example, if I use an ammonium nitrate of such fineness that not more than 17% by weight 45 passes a 60-mesh sieve, I obtain an explosive whose velocity of detonation is substantially lower than an explosive made with usual ammonium nitrate. The velocity of 50 this explosive will run from 1800 to 2600 meters per second, and on account of this low velocity the explosive is of great advan-

tage for work in which a slow explosive is desired, such, for example, as soft coal mining. When it is desired to obtain an explosive of especially low velocity of detonation, 55 it is of advantage to use ammonium nitrate which is in the form of rounded grains, or globules, instead of sharp, pointed particles, such as might be obtained by grinding ammonium nitrate or by certain methods of 60 crystallization.

While I have described my invention above in detail, I wish it to be understood that many changes may be made in the details thereof without departing from the 65 spirit of my invention.

By the term "relatively large", as applied to the size of the grains or particles in the claims, is meant grains of nitrate of ammonia substantially as large or larger than 70 grains of which not more than approximately seventeen per cent. by weight will pass through a sixty mesh sieve. By the term "relatively low velocity of detonation" appearing in the claims, is meant a velocity 75 of detonation substantially lower than twenty-seven hundred meters per second.

I claim:

1. An explosive having a relatively low velocity of detonation, comprising nitrate 80 of ammonia in relatively large particles.

2. An explosive having a relatively low velocity of detonation, comprising nitrate of ammonia in relatively large globular grains.

3. An explosive having a relatively low velocity of detonation and comprising nitrate of ammonia, nitroglycerin and an absorbent, the nitrate of ammonia being in the form of relatively large particles.

4. An explosive having a relatively low velocity of detonation, and comprising nitrate of ammonia, nitroglycerin, and an absorbent, the nitrate of ammonia being in the form of relatively large globular grains. 95

In testimony that I claim the foregoing I have hereunto set my hand.

CLIFFORD A. WOODBURY.

Witnesses:

C. R. MUDGE,  
FREDERICK LOREN GALLUP.